

# UNITED STATES PATENT OFFICE.

CHARLES BÖHM, OF NEW YORK, N. Y.

## PROCESS OF RENDERING LEATHER WATERPROOF.

SPECIFICATION forming part of Letters Patent No. 649,155, dated May 8, 1900.

Application filed January 17, 1900. Serial No. 1,723. (No specimens.)

*To all whom it may concern:*

Be it known that I, CHARLES BÖHM, a citizen of Germany, and a resident of New York city, county and State of New York, have invented a certain new and useful Improvement 5 in Processes of Rendering Leather Waterproof, of which the following is a specification.

This invention relates to a novel manner of treating leather so as to render it imper- 10 vious to water, oils, and acids. By my invention also the durability of the leather is increased and its liability to stretch is diminished. Thus leather treated according to my invention will be found of superior utility in 15 the various branches of manufacture—such as shoes, belting, trunks, harness, wearing-ap- parel, pocket-books, &c.

In carrying my invention into effect I proceed as follows:

20 First. I prepare a bath of about one (1) pound of wax and half an ounce of oil of mirbane, (nitrobenzol,) which is an oil sub- stance. After the wax has been melted in a hot-water bath over a fire the oily substance 25 is added and thoroughly stirred in. Into this heated bath the leather is immersed for from four to five hours, according to the degree of hardness of the leather under treatment. The oil of mirbane has the quality of com- 30 pletely combining with the wax without leav- ing any fatty deposit upon the leather after the latter has been subjected to the second bath. I have found that for the purposes of this invention oil of bergamot is an equiva- 35 lent of the oil of mirbane.

Second. A second bath is prepared com- posed of equal parts of alcohol and benzin, which is also slightly heated. The leather taken out of the first bath is immersed into the second bath and subjected to its action 40 for about half an hour. After removal it is dried in the fresh air and is then ready for use. The second bath will cause the wax to be removed clean from the surface of the leather, and practice has demonstrated that 45 by the process described the wax will be re- tained within the pores of the leather.

Leather prepared according to my inven- 50 tion will be pliable, impermeable to liquids, and of increased strength and durability, 55 and thus leather of a poor grade will be greatly improved in quality. So, also, the in- vention is particularly adapted for treating leather used for driving-belts and similar purposes, because it will become non-absorp- 55 tive to oil and will not stretch under ordinary tension.

What I claim is—

The process of treating leather, which con- 60 sists in subjecting it first to a bath of molten wax and nitrobenzol, then to a bath of alcohol and benzin, and finally drying the leather, substantially as specified.

Signed by me at New York city, county and State of New York, this 16th day of Jan- 65 uary, 1900.

CHARLES BÖHM.

Witnesses:

WILLIAM SCHULZ,  
F. V. BRIESEN.